

Aug. 5, 1952

F. M. CULPEPPER ET AL

2,605,502

PREPARATION OF FILAMENTARY MATERIAL

Filed Oct. 5, 1949



## UNITED STATES PATENT OFFICE

2,605,502

## PREPARATION OF FILAMENTARY MATERIAL

Frank M. Culpepper, Newark, N. J., and Lester W. Latta, Lynbrook, N. Y., assignors to Celanese Corporation of America, New York, N. Y., a corporation of Delaware

Application October 5, 1949, Serial No. 119,614

10 Claims. (Cl. 18-8)

**1**  
This invention relates to the preparation of filamentary material and relates more particularly to the preparation of filamentary material by the band spinning process.

In the preparation of filamentary material such as yarns, filaments, ribbon and the like by the band spinning process, a band of filament-forming material is entered at a constant rate, by means such as feed rollers, into a heated melting tube having a passageway extending therethrough of such size and shape as approximately to fit the band, which passageway leads to a spinning jet containing at least one spinning orifice. The filament-forming material melts and is brought to the proper temperature for spinning as it traverses the melting tube to the spinning jet and the molten filament-forming material is forced through the spinning orifice by the pressure developed by the incoming band, which acts as a continually-renewed piston. Among the filament-forming materials that may be spun in this manner are, for example, the polycarboxamides, polysulfonamides, polyurethanes, polytriazoles and the like.

We have found that in producing filamentary material by the band spinning process, there is a tendency for the band to jam in the feed mechanism or in the passageway, which jamming is highly objectionable since it interrupts the continuity of spinning. Moreover, when spinning is interrupted, the molten filament-forming material remaining in the melting tube tends to decompose or degrade so that the melting tube must be disassembled and cleaned before spinning can be resumed. In addition, we have found that during spinning the filament-forming material tends to decompose at a short distance, say 1 or 1.5 inches from the entrance to the passageway, and that the decomposition products which are formed tend to accumulate in and obstruct said passageway, requiring frequent interruptions to spinning for their removal.

It is an important object of this invention to provide a process and apparatus for preparing filamentary material by band spinning which will be free from the foregoing and other disadvantages and which will be especially simple in construction and efficient in operation.

A further object of this invention is the provision of a process and apparatus for the preparation of filamentary material by band spinning in which spinning may be carried on for extended periods of time without interruption.

Other objects of our invention, together with certain details of construction and combinations

**2**

of parts, will be apparent from the following detailed description and claims.

We have now discovered that the jamming of the band of filament-forming material in the feed mechanism results from a softening of the portion of the band between the feed rollers and the entrance to the melting tube produced by the heat reaching said band from the melting tube. If a considerable amount of softening takes place, 10 jamming will occur with a complete interruption in spinning. On the other hand, if only a limited amount of softening takes place, spinning may continue, but the band will be deformed, causing a variation in the rate at which the filament-forming material enters the melting tube, 15 which in turn will produce an objectionable variation in the denier of the filamentary material being produced.

To eliminate the jamming or deformation of 20 the portion of the band of filament-forming material between the feed rollers and the entrance to the melting tube, we provide a cooling means to prevent a softening of said band until after it has entered said melting tube. The cooling 25 means may, for example, take the form of a collar encircling the band and positioned between the melting tube and the feed rollers, through which collar a cooling medium such as water is circulated to carry away the heat emanating from the melting tube.

While the provision of a cooling means to prevent an increase in the temperature and a softening of the band of filament-forming material until after it has entered the melting tube eliminates the jamming or deformation of the band 35 in the feed rollers, it has no effect on the tendency of the band to jam in the passageway. We have discovered that the jamming of the band in the passageway results from the manner in which the band melts as it traverses said passageway. When the band enters the passageway and contacts the walls thereof, its outer surfaces begin to melt while its core remains solid. Then as the band passes farther into the passageway more of the filament-forming material on its outer surfaces melts and its core becomes plastic. The complete melting of the band takes place slowly when the same amount of heat is supplied to the band for the entire length of the passageway. As a result, the length of the plastic, but still unmelted, core of the band becomes so great that a very small obstruction to the movement of its tip is enough to halt the movement of the band and cause the band to jam progressively tighter and tighter in the passageway. When

a jam of this type takes place, it is not possible to move the band with thrusts of up to 300 pounds, although a thrust of only a few pounds is sufficient for spinning under normal conditions.

We have discovered that the jamming of the band of filament-forming material in the passageway may be eliminated by supplying a greater amount of heat to that portion of the passageway into which the band first enters than to the remainder of said passageway, so that the band will be melted rapidly and the molten filament-forming material will be brought to the proper temperature for spinning. This may be effected by positioning a number of heating elements along the length of the melting tube and raising the heating elements adjacent that portion of the passageway into which the band first enters to a higher temperature than the remainder of the heating elements. Alternatively, or in addition, the walls forming that portion of the passageway into which the band first enters may be made of higher thermal conductivity than the walls forming the remainder of the passageway. For example, the walls forming that portion of the passageway into which the band first enters may be of a different material and/or thinner in cross-section, while the walls forming the remainder of the passageway may be provided with a layer of insulating material. In general, it is desirable to melt the band of filament-forming material as rapidly as possible without employing temperature so high as to cause an appreciable decomposition of the filament-forming material.

During the spinning, the filament-forming material tends to decompose at a short distance from the entrance to the passageway although it remains at this point for only a very short interval of time. The products formed during the decomposition of the filament forming material accumulate in and obstruct the passageway, requiring frequent interruptions to spinning for their removal. We have discovered that the decomposition of the filament-forming material may be eliminated or minimized by passing a stream of a gas, such as nitrogen, which is chemically inert to the filament-forming material, over the entrance to the passageway to exclude atmospheric oxygen from contact with the heated band or the molten filament-forming material. By using this expedient, it is possible to carry on spinning for extended periods of time without interruption.

A preferred embodiment of our invention will now be described with particular reference to the accompanying drawing in which

Fig. 1 is an elevational view, partly in section, of the band spinning apparatus, and

Fig. 2 is a cross-sectional view, taken on the line 2-2 in Fig. 1 in the direction of the arrows.

Referring now to the drawing, the reference numeral 11 designates a guide member into which a band of filament-forming material (not shown) is entered. The guide member 11 leads the band of filament-forming material between feed wheels 12 and 13, at least one of which is positively driven by any suitable means (not shown), which grip the band and feed the same forward at a constant rate. To prevent slippage of the band between the feed wheels 12 and 13, the surface of one or both of said feed wheels may be serrated or otherwise roughened and the feed wheels may be spring-pressed against each other in a manner well understood in the art.

After passing between the feed wheels 12 and

13, the band enters a guide member 14 which directs the band into a passageway 15 of a collar 16 that is provided with a duct 17 through which a cooling medium is circulated. Upon leaving the passageway 15, the band enters a melting tube 18 having a passageway 19 of rectangular cross section extending the length thereof, which passageway 19 has a cross-section approximately equal to the cross-section of the band. As shown, the collar 16 is spaced from the guide member 14 and the melting tube 18. It is to be understood, however, that the collar 16 may be abutted against one or the other of said members. The melting tube 18 is provided with a number of heating elements, such as electric heating coils 21 which are positioned along the length of said melting tube and which may be individually controlled. There are provided also a series of thermocouples 22 to measure the temperature of the melting tube 18 along the length of the passageway 19. The signals from the thermocouples 22 may be employed to control automatically the magnitude of the current flowing to each of the several electric heating coils 21 so that the temperatures along the passageway 19 will remain constant at all times.

Adjacent the entrance to the passageway 19, there are provided a pair of opposed channels 23, which extend through the body of the melting tube 18 and intersect the passageway 19. A stream of a gas, such as nitrogen, which is inert to the filament-forming material, is entered into the channels 23 from any suitable source (not shown) through conduits 24. The incoming nitrogen flows to the atmosphere through the passageway 19 between the surfaces of the entering band and the walls of the melting tube 18, effectively excluding atmospheric oxygen from contact with the heated band or molten filament-forming material, and thereby eliminating or minimizing the decomposition of the filament-forming material.

From the passageway 19, the molten filament-forming material enters a well 25 in which a thermocouple 26 is positioned to measure the temperature of the filament-forming material immediately before it is spun. The molten filament-forming material then passes through a stainless steel filter screen 27 to remove any particles of foreign matter therefrom, following which the molten filament-forming material flows through the orifices (not shown) in the spinning jet 28. If desired, a sand filter may be placed above the stainless steel filter screen 27 further to filter the filament-forming material, in a manner well understood in the art. The outer or exposed surface of the spinning jet 28 may be given a high polish, which serves to reduce the heat radiated to the filamentary material from the surfaces of said jet and also to conserve the heat in the mass of molten filament-forming material contained within the well 25. The outer or exposed surface of the spinning jet 28 may be coated with a layer or film of silicone grease or graphite to make the jet self-starting when spinning is begun and also to aid in the removal of any deposits that accumulate on the surface of said jet during spinning. The filter screen 21 and the spinning jet 28 are held securely in position by means of a retaining ring 29, which is fastened to the body of the melting tube 18 in any suitable manner.

As the filament-forming material leaves the spinning jet 28, it tends to decompose and the decomposition products which are formed ac-

cumulate on the outer surface of said spinning jet. To prevent or minimize the decomposition of the filament-forming material, there may be provided a ring 31 supported on straps 32 and having a series of inwardly directed apertures 33 therein to which a stream of a gas, such as nitrogen, which is inert to the filament-forming material, is supplied from a suitable source (not shown) through a conduit 34. The stream of nitrogen blankets the outer surface of the spinning jet 28 and serves to prevent or minimize the decomposition of the filament-forming material. After cooling, the filamentary material may be passed through a humidifying chamber to increase its moisture content, lubricated and wound in package form, all as well understood in the art.

The following example is given to illustrate this invention further.

*Example*

The upper part of the melting tube 18 of the apparatus shown in the accompanying drawing is brought to a temperature of 290° C. and the lower part of said melting tube is brought to a temperature of 275° C. The passageway 19 is flushed with nitrogen and a band of a polycarboxamide prepared by the polymerization of hexamethylene diamine and adipic acid is entered into said passageway. Spinning starts easily and a 10 filament yarn having a total denier of 120 is spun at a speed of 665 meters per minute for an extended period of time without any jamming of the band between the feed rollers 12 and 13 or in the passageway 19 and without any accumulation of deposits at the entrance to said passageway.

While we have shown the passageway 19 as of rectangular cross-section, a passageway of other cross-section, such as circular or oval, for example, may also be employed, in which case the cross-section of the band of filament-forming material will be varied so as approximately to fit said circular or oval passageway. In addition, the cross-section of the passageway 19 need be approximately equal to that of the band only in the vicinity of the entering end of the melting tube 18, and the remainder of the passageway 19 may be of different cross-section from that of the band of filament-forming material.

It is to be understood that the foregoing detailed description is given merely by way of illustration and that many variations may be made therein without departing from the spirit of our invention.

Having described our invention, what we desire to secure by Letters Patent is:

1. In an apparatus for the preparation of filamentary material by the band spinning process, the combination with a melting tube having a passageway extending therethrough, of feed rollers for entering a band of filament-forming material into said passageway, said feed rollers being spaced from said melting tube and a collar encircling said band and positioned in the space between said feed rollers and said melting tube and spaced from said feed rollers and said melting tube, said collar having a duct therein for the passage of a cooling medium to prevent a softening of said band between the feed rollers and the entrance to the melting tube.

2. In an apparatus for the preparation of filamentary material by the band spinning process, the combination with a melting tube having a passageway extending therethrough, of feed

means for entering a band of filament-forming material into said passageway, cooling means for preventing a softening of said band between the feed means and the entrance to the melting tube, means for passing a stream of gas which is inert to the filament-forming material over the entrance to said passageway to exclude atmospheric oxygen from contact with the heated band or molten filament-forming material, and means for supplying a greater amount of heat to that portion of the passageway into which the band first enters than to the remainder of said passageway.

3. In an apparatus for the preparation of filamentary material by the band spinning process, the combination with a melting tube having a passageway extending therethrough, of feed rollers for entering a band of filament-forming material into said passageway, a collar encircling said band and positioned between said feed rollers and said melting tube, said collar having a duct therein for the passage of a cooling medium to prevent a softening of said band between the feed rollers and the entrance to the melting tube, a pair of opposed channels extending through the body of the melting tube and intersecting said passageway for the passage of a stream of gas which is inert to the filament-forming material over the surfaces of the band as it enters said passageway to exclude atmospheric oxygen from contact with the heated band or molten filament-forming material, and a plurality of individually controlled heating elements positioned along the length of said melting tube whereby a greater amount of heat may be supplied to that portion of the passageway into which the band first enters than to the remainder of said passageway.

4. In an apparatus for the preparation of filamentary material by the band spinning process, the combination with a melting tube having a passageway of rectangular cross-section extending therethrough, of feed rollers for entering a rectangular band of filament-forming material having a cross-section approximately equal to that of the passageway into said passageway, a collar encircling said band and positioned between said feed rollers and said melting tube, said collar having a duct therein for the passage of a cooling medium to prevent a softening of the band between the feed rollers and the entrance to the melting tube, a pair of opposed channels extending through the body of the melting tube, and intersecting said passageway for the passage of a stream of gas which is inert to the filament-forming material over the surfaces of the band as it enters said passageway to exclude atmospheric oxygen from contact with the heated band or molten filament-forming material, a plurality of individually controlled electrical heating coils positioned along the length of said melting tube whereby a greater amount of heat may be supplied to that portion of the passageway into which the band first enters than to the remainder of said passageway, a filter screen for removing extraneous foreign particles from the molten filament forming material, and a spinning jet having at least one spinning orifice for shaping the molten filament-forming material and having a polished outer surface for reducing the heat radiated therefrom.

5. In the preparation of filamentary material by the band spinning process, the steps which comprise forwarding a band of filament-forming material, passing the band into a first zone having an entering portion whose cross-section is

approximately equal to that of the band to melt the band, cooling the band before its entry into said heated zone to prevent a softening of the band before its entry into said heated zone, passing a stream of nitrogen over the entrance to said heated zone to exclude atmospheric oxygen from contact with the heated band or molten filament-forming material, passing the molten filament-forming material through a second zone to bring the molten filament-forming material to the proper spinning temperature, and supplying a greater amount of heat to said first zone than to said second zone.

6. In an apparatus for the preparation of filamentary material by the band spinning process, the combination with a melting tube having a passageway extending therethrough, of feed means, spaced from said melting tube, for entering a band of filament-forming material in said passageway, cooling means positioned in the space between said feed means and said melting tube and spaced from said feed means and said melting tube for preventing a softening of said band between the feed means and the entrance to the melting tube, and means, including a channel extending through the body of said melting tube and intersecting said passageway in said melting tube, for passing a stream of gas, which is inert to the filament-forming material, over the entrance to said passageway of said melting tube to exclude atmospheric oxygen from contact with the heated band or molten filament-forming material.

7. In an apparatus for the preparation of filamentary material by the band spinning process, the combination with a melting tube having a passageway extending therethrough, of feed means, spaced from said melting tube, for entering a band of filament-forming material in said passageway, cooling means positioned in the space between said feed means and said melting tube and spaced from said feed means and said melting tube for preventing a softening of said band between the feed means and the entrance to the melting tube, and means, including a pair of opposed channels extending through the body of said melting tube and intersecting said passageway in said melting tube, for passing a stream of gas, which is inert to the filament-forming material, over the entrance to said passageway of said melting tube to exclude atmospheric oxygen from contact with the heated band or molten filament-forming material.

8. In an apparatus for the preparation of filamentary material by the band spinning process, the combination with a melting tube having a passageway extending therethrough, of feed means, spaced from said melting tube, for entering a band of filament-forming material in said passageway, cooling means positioned in the space between said feed means and said melting tube and spaced from said feed means and said melting tube for preventing a softening of said

band between the feed means and the entrance to the melting tube, means for passing a stream of gas, which is inert to the filament-forming material, over the entrance to said passageway of said melting tube to exclude atmospheric oxygen from contact with the heated band or molten filament-forming material, and means for supplying a greater amount of heat to that portion of said passageway into which the band first enters than to the remainder of said passageway.

9. In an apparatus for the preparation of filamentary material by the band spinning process, the combination with a melting tube having a passageway extending therethrough, of feed means, spaced from said melting tube, for entering a band of filament-forming material in said passageway, cooling means positioned in the space between said feed means and said melting tube and spaced from said feed means and said melting tube for preventing a softening of said band between the feed means and the entrance to the melting tube, means, including a pair of opposed channels extending through the body of said melting tube and intersecting said passageway in said melting tube, for passing a stream of gas, which is inert to the filament-forming material, over the entrance to said passageway of said melting tube to exclude atmospheric oxygen from contact with the heated band or molten filament-forming material, and means for supplying a greater amount of heat to that portion of said passageway into which the band first enters than to the remainder of said passageway.

10. In the preparation of filamentary material by the band spinning process, the steps which comprise forwarding a band of filament-forming material, passing the band into a first zone to melt the band, cooling the band before its entry into said heated zone to prevent a softening of the band before its entry into said heated zone, passing a stream of nitrogen over the entrance to said heated zone to exclude atmospheric oxygen from contact with the heated band or molten filament-forming material, passing the molten filament-forming material through a second zone to bring the molten filament-forming material to the proper spinning temperature, and supplying a greater amount of heat to said first zone than to said second zone.

50 FRANK M. CULPEPPER.  
LESTER W. LATTA.

#### REFERENCES CITED

The following references are of record in the 55 file of this patent:

#### UNITED STATES PATENTS

| Number    | Name    | Date           |
|-----------|---------|----------------|
| 2,295,942 | Fields  | Sept. 15, 1942 |
| 2,359,013 | Tucker  | Sept. 26, 1944 |
| 2,367,173 | Martin  | Jan. 9, 1945   |
| 2,369,506 | Weibel  | Feb. 13, 1945  |
| 2,476,830 | Spencer | July 19, 1949  |